

# UNITED STATES PATENT OFFICE.

HERBERT B. COHO, OF MOUNT VERNON, NEW YORK.

## METALLIC COMPOUND.

Specification of Letters Patent. Patented May 11, 1915.

1,138,845.

Application filed September 22, 1914. Serial No. 862,960.

No Drawing.

*To all whom it may concern:*

Be it known that I, HERBERT B. COHO, a citizen of the United States, residing at Mount Vernon, in the county of Westchester 5 and State of New York, have invented new and useful Improvements in Metallic Compounds, of which the following is a specification.

My invention relates to a compound in which the basic elements are lead and copper 10 alloy held in suspension with needles (sulfid) antimony.

The object of my invention is to produce a compound of the character described that 15 may be readily commingled, economically produced, and which will result in a metallic compound that is susceptible of varied and extensive commercial utility.

A further object thereof is to produce an 20 alloy of lead and copper commingled with sulfid of antimony resulting in a very hard compound, and which when polished has the appearance of and may be used as a substitute for brass. And a still further object of 25 my invention is to produce a metallic compound of the character described in which the fluidity of the mixture is greatly increased to render same susceptible for small castings which are now made of brass.

To these ends, my invention includes the 30 combination of component ingredients to be hereinafter described and more particularly pointed out in the claims.

In the preparation of my compound, I 35 employ varied percentages of lead, copper and needles antimony (sulfid), the various proportions being determined by the hardness of the compound desired. The exact proportions of lead and copper are determined by the specific result desired and may 40 be varied within a wide range. For some purposes nine parts of lead may be employed with one part of copper, while in

other instances nine parts of copper and one part of lead is preferred. The proportions 45 of antimony sulfid employed is regulated by the degrees of hardness desired, as in a mixture of 50 pounds of copper and fifty pounds of lead from 5 pounds to 25 pounds of needles antimony (sulfid) may be used. It 50 has been found that for a bearing metal, 50 pounds of copper and 50 pounds of lead commingled with 5 pounds of antimony sulfid produces desirable results, while for imitation brass the proportion of copper 55 should be increased, and for packing metal the lead is increased and the copper decreased. The elements are thoroughly fused and commingled, and the resultant product may be readily cast and used as an efficient 60 substitute for brass castings and as an anti-friction bearing metal.

I have also found that by the addition of a desired quantity of tin in my compound, the same may be successfully employed as a 65 substitute for Babbitt metal with advantageous results.

When it is desired to increase the fluidity of the fused compound to facilitate its casting into small articles, a small addition of 70 sodium may be made in the preparation of the compound.

Having thus described my invention, what I claim as new and desire to be secured by 75 Letters Patent, is—

1. A metallic compound comprising lead and copper alloy commingled with needles antimony (sulfid).
2. A metallic compound comprising lead and copper alloy commingled and fused with 80 needles antimony (sulfid).

HERBERT B. COHO.

Witnesses:

H. D. BERESFORD,  
C. R. BABSON.